

# United States Patent [19]

Morin et al.

[11] Patent Number: 4,624,751

[45] Date of Patent: Nov. 25, 1986

[54] PROCESS FOR FIBER PLATING AND APPARATUS WITH SPECIAL TENSIONING MECHANISM

[75] Inventors: Louis G. Morin, Tarrytown, N.Y.; Robert E. Hoebel, Bristol, Conn.

[73] Assignee: American Cyanamid Company, Stamford, Conn.

[21] Appl. No.: 661,861

[22] Filed: Jul. 16, 1984

## Related U.S. Application Data

[63] Continuation of Ser. No. 507,619, Jun. 24, 1983, abandoned.

[51] Int. Cl.<sup>4</sup> ..... C25D 7/06; C25D 17/00

[52] U.S. Cl. ..... 204/28; 204/206

[58] Field of Search ..... 204/28, 207, 27, 206

## References Cited

## U.S. PATENT DOCUMENTS

3,061,534 10/1962 Jasperson ..... 204/28

|           |         |                              |          |
|-----------|---------|------------------------------|----------|
| 3,308,042 | 3/1967  | Lozano et al. ....           | 204/28   |
| 3,316,160 | 4/1967  | Uchida et al. ....           | 204/28   |
| 3,622,283 | 11/1971 | Sara ....                    | 29/183.5 |
| 3,807,996 | 4/1974  | Sara ....                    | 75/204   |
| 3,894,677 | 7/1975  | La Iacona ....               | 228/190  |
| 3,947,343 | 3/1976  | Delves-Broughton et al. .... | 204/207  |
| 4,132,828 | 1/1979  | Nakamura et al. ....         | 428/366  |
| 4,214,961 | 7/1980  | Anthony ....                 | 204/140  |
| 4,351,713 | 9/1982  | Hirt et al. ....             | 204/207  |
| 4,395,320 | 7/1983  | Kashashima et al. ....       | 204/206  |

## FOREIGN PATENT DOCUMENTS

1272777 5/1972 United Kingdom

Primary Examiner—Howard S. Williams

Attorney, Agent, or Firm—Michael J. Kelly; Edward A. Hedman

## ABSTRACT

A process and apparatus for metal plating fibers in which an array of tensioning rollers and contact rollers insure a direct tight path for the fiber and facilitate rapid replacement of the contact rollers when necessary.

21 Claims, 18 Drawing Figures





—  
FIG.



FIG. 3



FIG. 2



FIG. 4



5  
FIG.

FIG. 6



FIG. 8



FIG. 7





FIG. 9



FIG. 10



## FIG. II



FIG. 13



FIG. 14



FIG. 12



FIG. 5



FIG. 16



FIG. 17



FIG. 18

PROCESS FOR FIBER PLATING AND  
APPARATUS WITH SPECIAL TENSIONING  
MECHANISM

CROSS-REFERENCE TO RELATED  
APPLICATIONS

This application is a continuation of application Ser. No. 507,619, filed Jun. 24, 1983, now abandoned.

This application is related to APPARATUS AND PROCESS FOR CONTINUOUSLY PLATING FIBER, LOUIS G. MORIN, U.S. patent application Ser. No. 507,440, and CONTACT ROLLER MOUNTING ASSEMBLY and TENSIONING MECHANISM FOR ELECTROPLATING FIBER, ROBERT F. HOEBEL, U.S. patent application Ser. No. 507,612, both of which are being filed coincidentally with this application.

BACKGROUND OF THE INVENTION

1. Field of the Invention

This invention relates to metal coated filaments and to a process and an apparatus for their continuous production.

2. Description of the Prior Art

Filaments comprising non-metals and semi-metals, such as carbon, boron, silicon carbide, polyester, nylon, aramid, cotton, rayon, and the like, in the form of monofilaments, yarns, tows, mats, cloths and chopped strands are known to be useful in reinforcing metals and organic polymeric materials. Articles comprising metals or plastics reinforced with such fibers find wide-spread use in replacing heavier components made up of lower strength conventional materials such as aluminum, steel, titanium, vinyl polymers, nylons, polyester, etc. in aircraft, automobiles, office equipment, sporting goods, and in many other fields.

A common problem in the use of such filaments, and also glass, asbestos and others, is a seeming lack of ability to translate the properties of the high strength filaments to the material to which ultimate and intimate contact is to be made. In essence, even though a high strength filament is employed, the filaments are merely mechanically entrapped, and the resulting composite

40

45

50

55

60

65

The problems have been overcome in part by depositing a layer or layers of metals on the individual filaments prior to incorporating them into the bonding material, e.g., metal or plastic. Metal deposition has been accomplished by vacuum deposition, e.g., the nickel on fibers as described in U.S. Pat. No. 4,132,828; and by electroless deposition from chemical baths, e.g., nickel on graphite filaments as described in U.S. Pat. No. 3,894,677; and by electrodeposition, e.g., the nickel electrodeplating on carbon fibers as described in Sara, U.S. Pat. No. 3,622,283 and in Sara, U.S. Pat. No. 3,807,966. When the metal coated filaments of such procedures are twisted or sharply bent, a very substantial quantity of the metal flakes off or falls off as a powder. When such metal coated filaments are used to reinforce either metals or polymers, the ability to resist compressive stress and tensile stress is much less than what would be expected from the rule of mixtures, and this is strongly suggestive that failure to efficiently reinforce is due to poor bonding between the filament and the metal coating.

5

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

5005

5010

5015

5020

5025

5030

5035

5040

5045

5050

5055

5060

5065

5070

5075

5080

5085

5090

5095

5100

5105

5110

5115

5120

5125

5130

5135

5140

5145

5150

5155

5160

5165

5170

5175

5180

5185

5190

5195

5200

5205

5210

5215

5220

5225

5230

5235

5240

5245

5250

5255

5260

5265

5270

5275

5280

5285

5290

5295

5300

5305

5310

5315

5320

5325

5330

5335

5340

5345

5350

5355

5360

5365

5370

5375

5380

5385

5390

5395

5400

5405

5410

5415

5420

5425

5430

5435

5440

5445

5450

5455

5460

5465

5470

5475

5480

5485

5490

5495

5500

5505

5510

5515

5520

5525

5530

5535

5540

5545

5550

5555

5560

5565

5570

5575

5580

5585

5590

5595

5600

5605

5610

5615

5620

5625

5630

5635

5640

5645

5650

5655

5660

5665

5670

5675

5680

5685

5690

5695

5700

5705

5710

5715

5720

5725

5730

5735

5740

5745

5750

5755

5760

5765

## SUMMARY OF THE INVENTION

It is a basic object of the present invention to provide fibers formed of a conductive semi-metallic core with metallic coatings.

It is another object of the present invention to provide a process in which the electroplating of the fibers is effected under high voltage electroplating conditions.

Further, it is an object of the present invention to provide a process and apparatus which will efficiently and rapidly coat fibers with metallic coatings and facilitate the cleaning and collecting of the finished product.

In accordance with the present invention, apparatus has been provided in which a plurality of fibers can be simultaneously plated efficiently with a metal surface and thereafter cleaned and reeled for use in a variety of end products.

The apparatus is a continuous line provided generally with a pay-out assembly adapted to deliver a multiplicity of fibers to an electrolytic plating bath. The line includes a pre-treatment process, after which the metal-plating is performed in a continuous process by the passage of the clean fibers through an electrolyte under high voltage conditions. Means are provided to cool the fibers during the passage from the contact roll associated with the electrolytic tank and the electrolyte bath.

Further, the fibers pass over contact rollers into the electrolyte. The line includes an assembly of tensioning rollers that serve to insure a tight direct line of the fiber from the contact roller to the electrolyte.

The tensioning assembly is comprised of a plurality of driven rollers over which the fibers pass, and the path of the fibers are reversed to create tension. The tensioning rollers are driven independently of the drive for the processing apparatus and at a speed equal to or less than the speed of the fiber. The speed is determined by visual inspection.

The contact rollers are located in close proximity to the surface of the electrolyte, and by virtue of the processing conditions require frequent change. As a result the contact rollers are mounted on fixed aligned mounts. The mounts both carry support bushings having an outside diameter equal to the inside diameter of the contact roller.

## DESCRIPTION OF THE DRAWINGS

The invention will be more readily understood when viewed in association with the following drawings wherein:

FIG. 1 is a schematic view of the overall process of the subject continuous electrolytic plating process except for the pay-out assembly.

FIG. 2 is an elevational view of the pay-out section arranged specifically to simultaneously deliver a multiplicity of fibers to the electrolytic plating operation.

FIG. 3 is a plan view of the pay-out assembly of FIG. 2.

FIG. 4 is an isometric view of the wetting and tensioning rollers between the pay-out and electrolytic bath.

FIG. 5 is an elevational view of one electrolytic tank.

FIG. 6 is a plan view of the tank of FIG. 5.

FIG. 7 is a sectional elevational view through line 10-10 of FIG. 5.

FIG. 8 is an isometric view of the commutation fingers.

FIG. 9 is an isometric view of one contact roller in association with the means for providing coolant to the

fibers and a current carrying medium from the contact roller to the bath.

FIG. 10 is an elevational view of a section of the electrolytic tank depicting an anode basket.

FIG. 11 is a schematic of the electrolytic coolant conductor and a contact roller.

FIG. 12 is a sectional elevational view of a contact roller of the process assembly.

FIG. 13 is a detail of the end cap of the roller of FIG. 12.

FIG. 14 is a partial detail of the opposite end of the roller of FIG. 12.

FIG. 15 is a view of the electrical system of the present invention.

FIG. 16 is a drawing of the mechanism for synchronously driving the apparatus of the subject invention.

FIG. 17 is a plan view through line 28-28 of the section of FIG. 16.

FIG. 18 is a side elevational view of the roller assembly in the drying section of the system.

## DESCRIPTION OF THE PREFERRED EMBODIMENT

The process and apparatus of the present invention are directed to providing an efficient and complete means for metal-plating non-metallic and semi-metallic fibers.

The process of the invention relies on the use of very high voltage and current to effect satisfactory plating.

As a result of the high voltage and current, an apparatus has been developed that can produce high volumes of plated material under high voltage conditions.

The process of the present invention and the apparatus particularly suitable for practicing the process of the invention are described in the preferred embodiment in which the specified fiber to be plated is a carbon or graphite fiber and the plating metal is nickel. However, the process and apparatus of the present invention are suitable for virtually the entire spectrum of metal-plating of non-metallic and semi-metallic fibers.

The overall process and schematic of the apparatus except for the pay out assembly are generally shown in FIG. 1. The operative process includes in essence, a pay-out assembly for dispensing multiple fibers in parallel, tensioning assembly 6, a pre-treatment section 8, a plating facility 10, a rinsing station 12, a drying section 14 and take-up reels 16.

More particularly, the pre-treatment section 8 shown generally in FIG. 1 includes a tri-sodium phosphate cleaning section 26 and an associated washing-tee 28, rinse section 30 and associated washing-tees 32 and 32A, a hydrochloric acid section 34 and associated tee 36, and rinse section 38 with associated washing-tees 40 and 40A. The plating facility 10 is comprised of a plurality of series arranged electrolyte tanks shown illustratively in FIG. 1 as tanks 18, 20, 22 and 24, each of which is charged with current by a separate rectifier, better seen in FIGS. 5 and 15. The rinsing section 12, shown generally in FIG. 1 is comprised of tank and tee assemblies similar to the pre-treatment apparatus. An arrangement of cascading tanks 42 and tees 44, 44A and 44B cycle rinse solution of water and electrolyte over the fibers 2. Thereafter, clean water is passed over the fibers 2 in the rinse section 46 provided with tanks and washing-tees 48 and 48A. The rinsed fiber 2 is then passed through section 50 wherein it is first air blasted in chamber 53 and then steam treated in section 55 to produce an oxide surface on the metal plate. The process is com-

pleted by passage of the metal plated fiber 2 through the drying unit 14 and reeling of the finished fibers on take-up reels 17 in the reeling section 16.

As seen generally in FIG. 1, the apparatus is provided with means to convey the fibers 2 through the system rapidly without abrading the fibers 2. The combination of strategically located guide rollers 51, tension rollers 90 comprising tensioning assembly 6, force imposing rollers in the drying section 14 and a synchronous drive assembly shown in FIG. 16 rapidly conveys the fibers 2 through the apparatus without abrasion of the fibers 2.

The operation begins with the pay-out assembly 4 shown in FIGS. 2 and 3. Functionally, the fibers 2 from the pay-out assembly 4 are delivered over a guide roller 5 through the tensioning rollers 90 of tensioning assembly 6 to the pretreatment section 8.

As best seen in FIGS. 2 and 3, the pay-out assembly 4 is comprised of a frame 52 on which the pay-out rollers 54 are mounted. The pay-out rollers 54 are mounted on the frame 52 on a rail 56 and a rail 58. The rollers 54 on rail 56 are arranged to pay-out the fibers 2 to the electroplating system while the rail 58 is an auxiliary rail adapted to mount the spare rollers 54 available to provide alternate duty. A rail 60 mounts guide rollers 62 over which the fibers 2 from the pay-out rollers 54 travel to reach the tensioning rollers 90 of tensioning assembly 6. As best seen in FIG. 2, the fibers 2 extend from the respective rollers 54 over individual guide roller 62 associated with a particular roller 54 to the common guide roller 5 and into the tensioning roller assembly 6. Guide bars 59 are provided to guide fibers 2 from the pay-out rollers 54 to the associated guide rollers 62.

As seen in FIG. 3, the guide rollers 62 are aligned adjacent to each other to avoid interference between the fibers 2 as a plurality of fibers 2 are simultaneously delivered to the system to be treated and plated.

The pay-out assembly 4 delivers the fibers 2 over a guide roller 5 to a wetting roller 80 and then to the tensioning rollers 90. A wetting tub 84 is provided with water which wet the fibers 2 and enables suitable and more efficient cleaning and rinsing of the fibers 2 during pre-treatment. The tensioning rollers 90 seen in FIG. 1 shown in more detail in FIG. 4.

The tensioning assembly 6 comprise an assembly of five rollers 90, all of which are driven through a single continuous chain 87 by a common source such as a variable speed motor 92. Each roller 90 is mounted on a shaft 89 which also mounts a fixed gear 91 around which the chain 87 is arranged. Idler rollers 97 are also arranged to engage the chain 87. A gear 93 extending from the shaft 95 of the variable speed motor 92 drives the continuous chain 87 through a chain 101 and a gear 103 fixed to the shaft 89 of a roller 90. It is necessary that tension be provided to the fibers 2 at a location in the line upstream of the first plating contact roller. The plating contact roller and the fibers 2 must be in tight contact to facilitate the operation at the high voltage and high current levels necessary for the process. With tight contact, low resistance is provided between the fibers 2 and the contact rollers, thus the high current passing through the system circuit will not overload the fibers 2 causing destruction of the fibers. As a result, the tension roller assembly 6 is located upstream of the electroplating tanks 18, 20, 22, 24 (FIG. 1) to provide that tension. On the other hand, the fibers should be subjected to as little drag as possible. Inherent in the fibers 2 is the tendency to separate at the surface and accumu-

late fuzz. The variable drive motor 92 is coupled to all five of the rollers 90 to provide variable speed for the rollers at some speed equal to or less than the speed of the fibers 2. At carefully controlled speeds the necessary tension is provided without causing fuzz to accumulate on the fibers. The apparatus and process are designed to afford a tension roller assembly 6 in which the tension rollers 90 travel at a slower speed than the fibers 2. The tension on the fibers 2 is maintained by varying the speed of the tension roller 90 in response to visual determination of the tension.

The pre-treated fibers 2 are next electroplated. As seen in FIG. 1, a plurality of electroplating tanks 18, 20, 22 and 24 are provided in series. Under the high voltage-high current conditions of the process, the series arrangement of electroplating tank 18, 20, 22 and 24 afford means for providing discrete voltage and current to the fibers 2 as a function of the accumulation of metal-plating on the fibers 2. Thus, depending on the amount of metal-plating on the fibers 2, the plating voltage and current can be set to levels most suitable for the particular resistance developed by the fiber and metal.

The electrolytic plating tank 18 is shown in FIGS. 5, 6 and 7 and is identical in structure to the plating tanks 20, 22 and 24 shown in FIG. 1. The tank 18 is arranged to hold a bath of electrolyte. The tank 18 has mounted therewith contact rollers 100 and anode support bars 102 which are arranged in the circuit. The contact rollers 100 receive current from the bus bar 104 and the anode support bars 102 are connected directly to a bus bar 106. Each of the plating tanks 18, 20, 22 and 24 are provided with similar but separate independent circuitry as seen in FIG. 15. The anode support bars 102 have mounted thereon anode baskets 110 arranged to hold and transfer current to nickel or other metal-plating chips.

Each tank 18, 20, 22 and 24 is also provided with heat exchangers 114 to heat the electrolyte bath to reach the desirable initial temperature at start-up and to cool the electrolyte during the high intensity current operation.

The tank 18 is provided with a well 103 defined by a solid wall 105 in which a level control 107 is mounted and with a recirculation line 109. The recirculation line 109 includes a pump 111 and a filter 113 and functions to continuously recirculate electrolyte from the well 103 to the tank 18. Under normal operating conditions recirculated electrolyte will enter the tank 18 and cause the electrolyte in the tank to rise to a level above the wall 105 and flow into the well 103. When electrolyte has evaporated from the tank the level in the well will drop and call for make-up from the downstream rinse section 12.

The tank 18 is also provided with a line 132 and pump 134 through which electrolyte is pumped to a manifold 128 that delivers the electrolyte to the spray nozzle 130 above the contact rollers 100.

As shown in more detail in FIG. 10, the fibers 2 pass over the contact rollers 100 and around idler rollers 112 located in proximity to the bottom of the tank. The idler rollers 112 are provided in pairs around which the fibers 2 pass to move into contact with the succeeding contact roller 100.

The rollers 100 in the tank 18 communicate with the bus bar 104 through contact member 118. The detail of the contact member 118 seen in FIG. 8 shows that the contact members 118 are formed of a bar 120 and a plural array of fingers 122 and 124 that together provide

the positive contact over a sufficiently large area on the contact roller 100 to avoid creating a high resistance condition at the point of contact. The fingers 122 and 124 are resiliently mounted on the bar 120 and by the nature of the material, are urged into contact with the contact roller 100 at all times.

Thus, a high strength positive electrical contact assembly is provided for an environment wherein conventional brush contacts cannot serve well.

The high voltage-high current process of the present invention is further facilitated by means for protecting the fibers 2 during the passage between the electrolyte bath and the various contact rollers. The system includes the recirculating spray system 126 shown generally in FIGS. 5 and 6 through which electrolyte is recycled from the plating tanks and sprayed through the spray nozzles 130 on the fibers 2 at contact points on the contact rollers 100.

The spray nozzles 130 are arranged with two parallel tubular arms 136 and 138 having nozzle openings 139 located on the lower surfaces thereof.

One tubular arm 136 of the spray nozzle 130, is arranged to direct electrolyte tangentially on the fibers 2 at the point at which the fibers 2 leave the contact roller 100. The other tubular arm 138 of the spray nozzle 130 is arranged to deliver electrolyte directly on the top of the contact roller 100 at the point at which the fiber 2 engages the contact roller 100. As previously indicated, it is vital that sufficient tension be applied on the fibers 2 to insure that the fibers 2 are maintained in a tight direct line between the contact rollers 100 and the idler rollers 112. The need for a tight line is to assure that the low contact resistance suitable for current travel is available with high conductivity through the fibers 2 from the contact rollers 100 to the electrolyte bath. The electrolyte which is recirculated over the contact rollers 100 and the fibers 2 provide a parallel resistor in the circuit and serve to cool the fibers 2.

It is known that the fibers 2 being plated have a low fusing current, such as 10 amps for a 12K tow of about 7 microns in diameter. However, the process of the present invention requires about 25 amps between contacts or about 125 amps per strand in each tank.

Furthermore, both contact resistance and anisotropic resistance must be overcome. The contact resistance of 12K tow of about 7 microns on pure clean copper is about 2 ohms, thus at 45 volts twenty-two and one half amps are required before any plating can occur. The anisotropic resistance is 1,000 times the long axis. Thus, the total contact area must be 1,000 times the tow diameter, which for 7 microns is 0.34 inches. Practice has taught that one-half inch of contact will properly serve the electrical requirement of the system when plating 7 micron tow, hence two inch contact rollers 100 are used. It is also vital that the contact rollers 100 be located at a specified distance above the electrolyte bath to enable the system to operate at the high voltages necessary to achieve the plating of the process. In practice, it has been found that the contact rollers 100 should be located two inches from the electrolyte bath when voltages of 16 to 25 volts are applied. Further, it has been found that recirculation of about 2 gallons per minute per contact roller traveling at about 1½ to 25 ft./min. will properly cool the fiber and provide a suitable parallel resistor when above 5,000 amps are passed through the system.

The electrolyte in the process is a solution constituted of eight to ten ounces of metal, preferably in the form of

NiCl2 and NiSO4 per gallon of solution. The pH of the solution is set at 4 to 4.5 and the temperature maintained between 145° and 150° F. Recirculation of the electrolyte through the spray nozzles 130 at the desired rate requires that the nozzle openings be 3/32 inches in diameter on ½" centers over the length of each tubular arm 136 and 138. The presence of electrolyte on the fibers is vital, but care is taken to avoid excessive electrolyte otherwise the contact rollers will become subjected to the plating occurring in the electrolyte.

The contact rollers 100 are shown in detail in FIGS. 12-14. Each contact roller 100 is located in close proximity to the electrolyte in the plating tanks and each is adapted to transmit high current through the system in a high intensity voltage environment. The contact roller 100 thus is designed for continual replacement. The contact roller 100 is provided with fixed end mounting sections 170 and 172 which hold a cylindrical copper tube 174. The cylindrical copper tube 174 is arranged to contact the commutator fingers 122-124 and deliver current through both the fibers 2 and recycled electrolyte to the electrolyte bath. The copper tube 174 is formed of conventional type L copper which must be able to carry 350 amperes. The diameter of the tubing is critical in that the diameter dictates the contact surface for the fibers 2 and the distance that the contact roller 100 will be from the electrolyte surface. As a result, the mounts 170 and 172 are fixedly arranged in alignment with each other to releasably support the tube 174 of the contact roller 100. The mount 170 is provided with a bearing support 176 through which a screw mount 178 passes. The screw mount 178 rotatably supports the copper tube 174 on a bushing support 180 and has the capacity to release the copper tube 174 upon retraction of the bushing support 180 by withdrawing the screw 178. The mount 172 includes a bushing support 182 on which a detent 184 is formed. Each copper tube 174 is provided with a notched mating slot 186 to fit around the detent 184 and effect positive attachment of the copper tube 174 to the bushing support 182 thereby obviating any uncertainty in alignment and facilitating dispatch in replacing each copper tube section 174.

The overall electrical system 188 of the process and apparatus is shown schematically in FIG. 15 wherein the capacity for discrete application of voltage and current to each electrolytic tank 18, 20, 22, 24 can be seen. Conventional rectifiers 189, 191, 193 and 195 are arranged as a D.C. power source to deliver current to the respective contact rollers 100 on each electrolytic tank. Bus bars 104, 194, 196, 198 are shown for illustration extending respectively from the rectifiers 189, 191, 193 and 195 to one of the six contact rollers 100 on the electrolytic tanks 18, 20, 22 and 24. However, all six contact rollers 100 on each electrolytic tank are directly connected to the same bus bar. Bus bars 106, 202, 204 and 206 are shown extending respectively from the same rectifiers 189, 191, 193 and 195 through cables 208 to one anode support bar 102 mounted on the electrolytic tanks 18, 20, 22 and 24. Again the respective anode bus bars contact each anode support bar 102 mounted on each electrolytic tank connected to the bus bar.

As a result of the arrangement, discrete high voltage can be delivered to each electrolytic tank 18, 20, 22, 24 as a function of the metal plating on the fibers 2 in each electrolytic tank.

Practice has taught that the voltage in the first electrolyte tank 18 should not be below 16 volts and seldom be below 24 volts. The voltage in the second tank 20

should not be below 14 volts and the voltage in the third electrolyte tank 22 should not be below 12 volts.

Illustratively, fibers 2 have been coated in a system of three rectifier-electrolyte tank assemblies, rather than the four shown in FIGS. 1 and 15 under the following conditions wherein excellent coating has resulted:

| RECTIFIER | 189   | 191   | 193   |
|-----------|-------|-------|-------|
| AMPS      | 1,400 | 1,400 | 1,400 |
| VOLTS     | 45    | 26    | 17    |

10

The nickel metal coated fibers 2 produced under these conditions have the following properties and characteristics:

Filament Shape: Round (but dependent on graphite fiber)

Diameter: 8 microns

Metal Coating: Approximately 0.5 microns thick, about 50% of the total fiber weight.

Density: 2.50-3.00 grams/cm.<sup>3</sup>

Tensile Strength: Up to 450,000 psi

Tensile Modulus: 34 M psi

Electrical: 0.008 ohms/cm. (12K tow)

Conductivity: 0.10 ohms/1000 strands/cm.

After the nickel plating has occurred, the fully plated fibers 2 are delivered to the rinsing section seen in FIG. 1.

The drag-out section 42 and rinse section 46 are arranged with tanks to accumulate the discharge from the tees 44, 44A, 44B, 48 and 48A and both neutralize the discharge for waste disposal and provide a repository for accumulation of make-up for the electrolyte tanks 18, 20, 22 and 24.

The apparatus of the present invention is arranged for synchronous operation as shown in FIGS. 16-18. A motor 222 is provided to insure that the contact rollers 100 and the guide rollers 51 rotate at the same speed to avoid abrading the fibers 2.

The motor 222 directly drives an assembly of rollers 223 arranged to effect a capstan. The rollers 223 are located in the dryer 14 and as best seen in FIG. 18 cause the fiber to reverse direction six times. The reversal in direction is sufficient to impose a force on the fibers 2 that will pull the fibers through the apparatus without allowing slack.

In addition, the motor 222 is connected by a gear and chain assembly to drive each contact roller 100 and each guide roller 51 at the same speed.

In essence, the gear and chain assembly is comprised of guide drive assemblies 225, best seen in FIG. 17 and contact roller drive assemblies 227. Each guide drive assembly 225 includes drive transmission gear 230 mounted on shafts 231, a gear 224 fixedly secured to the guide roller 51 and a chain 233 that engages the gears 230 and 224.

The contact roller drive assembly includes drive transmission gear 239 mounted on the shafts 231 common to the gears 230, a gear 241 fixedly secured to each contact roller 100 and a chain 243 that engages both gears 239 and each of the gears 241 on the six contact rollers 100 associated with each electrolyte tank.

The location of the capstan rollers 223, seen in FIG. 18, in the dryer 14 enhances drying. The flat surface and force applied to the fibers 2 spreads the fibers and thereby accelerates drying.

The system also includes a variable speed clutch override drive motor 219 for the take-up reels 17. The force generated by the variable torque motor 219 pro-

vides the force to draw the fiber 2 through the system. However, the capstan rollers 223 provide a means to isolate the direct force imposed on the fibers 2 at the take-up reels 17 from the fibers 2 upstream of the capstan rollers.

What is claimed is:

1. A process for electroplating fiber comprising:

(a) continuously passing the fiber over a contact into an electrolyte solution in a tank in which a metal anode is immersed;

(b) passing D.C. current through the fibers to the anode; and

(c) imposing a tension on the fiber by passing the fiber over an array of tension rollers in a path that reverses the direction of the fiber and rotating the tension rollers in the direction of the fiber at a speed equal to or less than the speed of the fiber to insure a direct tight path than the speed of the fiber to insure a direct tight path from the fiber at the contact point to the electrolyte in the tank, whereby metal from the anode migrates to the fiber and is bonded thereto.

2. A process as in claim 1 wherein the tension is imposed on the fiber upstream of the contact.

3. A process as in claim 1 wherein the contact is a contact roller.

4. A process as in claim 3 further comprising the step of driving the contact roller in the same direction in which the fiber is traveling.

5. A process for electroplating fiber comprising:

(a) continuously passing the fiber over a contact into an electrolyte solution in a tank in which a metal anode is immersed;

(b) passing D.C. current through the fibers to the anode; and

(c) imposing a tension on the fiber by passing the fiber over an array of tension rollers in a path that reverses the direction of the fiber and rotating the tension rollers in the direction of the fiber at a speed equal to or less than the speed of the fiber to insure a direct tight path from the fiber at the contact point to the electrolyte in the tank, whereby metal from the anode migrates to the fiber and is bonded thereto and wherein the speed of the tension roller is regulated as a function of the tension of the fiber.

6. An apparatus for metal plating fibers, comprising:

(a) a D.C. rectifier;

(b) an electrolyte tank to which the rectifier delivers current;

(c) electrolyte in the electrolyte tank;

(d) a metal anode in the electrolyte;

(e) an electrolyte sprayed contact member immediately above the electrolyte surface;

(f) means for continuously passing fiber through the electrolyte;

(g) means for delivering D.C. current from the rectifier through the fibers to the electrolyte;

(h) means for maintaining tension on the fiber to insure a direct tight path from the fiber at the contact point to the electrolyte in the tank wherein the means for maintaining tension on the fiber is an array of tensioning rollers located upstream of the contact member over which the fibers pass to reverse direction; and

(i) means to drive the array of roller simultaneously at the same speed in the direction of the fiber at a speed equal to or less than the speed of the fiber.

7. An apparatus as in claim 6 wherein the means to drive the rollers is comprised of a gear on the shaft of each gear, and a variable speed motor coupled to the continuous chain to drive the chain.

8. An apparatus as in claim 7 wherein the contact member is a contact roller and further comprising means to rotate the contact roller in the direction of the fiber at the speed of the fiber.

9. An apparatus as in claim 8 wherein the array of tensioning rollers is comprised of five rollers.

10. A process for electroplating fiber comprising:

(a) continuously passing the fiber over a contact into an electrolyte solution in a tank in which a metal anode is immersed;

(b) passing D.C. current through the fibers to the anode; and

(c) imposing tension variably on the fiber between the contact point and the electrolyte in the tank, whereby metal from the anode migrates to the fiber and is bonded thereto.

11. A process as in claim 10 wherein the tension is imposed variably on the fiber upstream of the contact.

12. A process as in claim 11 wherein the tension is imposed variably by the steps of passing the fiber over an array of tension rollers in a path that reverses the direction of the fiber and rotating the tension rollers in the direction of the fiber at a variable speed equal to or less than the speed of the fiber.

13. A process as in claim 12 wherein the speed of the tension roller is regulated as a function of the tension of the fiber.

14. A process as in claim 10 wherein the contact is a contact roller.

15. A process as in claim 14 further comprising the step of driving the contact roller in the same direction in which the fiber is traveling.

16. An apparatus for metal plating fibers, comprising:

(a) a D.C. rectifier;

(b) an electrolyte tank to which the rectifier delivers current;

(c) electrolyte in the electrolyte tank;

(d) a metal anode in the electrolyte;

(e) an electrolyte sprayed contact member immediately above the electrolyte surface;

(f) means for continuously passing fiber through the electrolyte;

(g) means for delivering D.C. current from the rectifier through the fibers to the electrolyte; and

(h) means for maintaining tension variably on the fiber between the contact member and the electrolyte in the tank.

17. An apparatus as in claim 16 wherein the means for maintaining tension variably on the fiber is an array of tensioning rollers located upstream of the contact member over which the fibers pass to reverse direction.

18. An apparatus as in claim 17 further comprising means to drive the array of rollers simultaneously at the same speed in the direction of the fiber at a speed equal to or less than the speed of the fiber.

19. An apparatus as in claim 18 wherein the means to drive the rollers is comprised of a gear on the shaft of each tensioning roller, a continuous chain passing over each gear, and a variable speed motor coupled to the continuous chain to drive the chain.

20. An apparatus as in claim 19 wherein the contact member is a contact roller and further comprising means to rotate the contact roller in the direction of the fiber at the speed of the fiber.

21. An apparatus as in claim 20 wherein the array of tensioning rollers is comprised of five rollers.

\* \* \* \* \*